

## UNITED STATES PATENT OFFICE

2,061,267

## PREPARATION OF LEAD-SODIUM-MAGNESIUM ALLOYS

Frederick Baxter Downing, Carneys Point, Louis  
Samuel Bake, Penns Grove, and Alfred E. Par-  
melee, Carneys Point, N. J., assignors to E. I.  
du Pont de Nemours & Company, Wilmington,  
Del., a corporation of Delaware

No Drawing. Application November 16, 1934,  
Serial No. 753,301

4 Claims. (Cl. 75—167)

This invention relates to the preparation of lead-sodium-magnesium alloys.

An alloy comprising 10% sodium, 89.95% to 89.00% lead and 0.05 to 1.00% magnesium is described in an application of F. B. Downing and L. S. Bake, Ser. No. 708,248 filed January 25, 1934. A process employing this alloy is described and claimed in an application of Downing and Bake, Ser. No. 613,260, filed May 24, 10 1932. These applications of Downing and Bake disclose that the presence of a small amount of magnesium, in a lead-monosodium alloy employed for the manufacture of tetraethyl lead, has a marked effect upon the operation, in that 15 the yields are increased and the amount of unconverted alloy is decreased. When no magnesium is present with consequent high unconverted alloy present, the residues, during steam distillation, tend to ball up and cause difficulty in discharging the still. If magnesium is present, 20 the residual lead, after the distillation, tends to be finely divided and is easily discharged.

There are two general methods of preparing the ordinary lead-monosodium alloy. The first method consists in placing the required amount of lead and sodium in a pot and applying heat thereto until the reaction takes place to form PbNa. The reaction of lead and sodium to form the lead-sodium alloy is exothermic. When this method is practiced, enough heat is liberated to 25 raise the temperature of the alloy to from 500 to 670° C. At these high temperatures, there is a very strong tendency for the sodium to distill off and, if great care is not taken, the resulting 30 alloy will contain less than 10% sodium. This is a decidedly undesirable result as, if the amount of sodium varies as much as 0.1 to 0.2% below or above 10%, the alloy will not produce the maximum yields of tetraethyl lead. Magnesium 35 has a melting point of about 651° C. Accordingly, magnesium may be dissolved in the alloy by this method as the magnesium is soluble in the lead sodium alloy at such high temperatures. However, such method involves the problem of avoiding distillation of sodium from the 40 alloy.

The second method of preparing lead-monosodium alloy, and the method which is more generally employed at the present time, consists 45 either in adding molten sodium to molten lead or molten lead to molten sodium at the desired rate with stirring in a pot jacketed with molten diphenyl. In this process, the rate of addition of one ingredient to the other may be so controlled that the temperature within the pot does

not exceed 400° C. At this temperature, there is little tendency for the sodium to distill off and, furthermore, such temperatures are necessary to prevent decomposition of the diphenyl. Diphenyl starts to decompose at about 400° C. but such decomposition does not become serious until temperatures of about 410° C. and above are reached. However, at the temperature of about 400° C., it was found that, when magnesium was added to the alloy, it did not go into 10 solution in the alloy but remained floating on the surface of the molten alloy.

An object of the present invention is to provide a method for preparing lead-sodium-magnesium alloys such as are disclosed in the hereinbefore identified applications of Downing and Bake. A further object is to provide a method whereby such an alloy can be prepared at temperatures not in excess of 400° C. Other objects 15 are to advance the art. Still other objects 20 will appear hereinafter.

These objects may be accomplished in accordance with our invention which comprises fusing the magnesium with at least a major proportion of the lead to produce a lead-magnesium alloy which may be melted and added to the molten sodium or to which molten sodium 25 may be added.

Our invention is based upon the discovery that lead-magnesium alloys decrease in their melting points with increasing amounts of magnesium until a minimum melting point of approximately 250° C. is reached, when the alloy contains about 3% of magnesium. When the percent of magnesium is increased above this 30 point, the melting point gradually rises to 551.3° C. at 19.06% magnesium at which point only PbMg<sub>2</sub> is present. The melting point then decreases to 468° C. at approximately 35% magnesium and then increases gradually to 651° C., 40 when pure magnesium is present. On the way up from the minimum of 250° C., the melting point curve crosses the 400° C. line at approximately 8.7% magnesium. Accordingly, it is evident that, if any lead magnesium alloy containing up to 8.7% of magnesium is added to a molten lead-sodium alloy at 400° C., fusion of the lead-magnesium alloy will be effected and a homogeneous mixture of the magnesium will be obtained.

We have found that lead-magnesium alloys having a melting point up to about 500° C. may be melted and then added to molten sodium or a molten lead-sodium alloy and such lead-magnesium alloy will dissolve in the sodium or

lead-sodium alloy and form a homogeneous mixture therewith. According to the broader aspects of our invention, therefore, we contemplate preparing lead-magnesium alloys containing such a proportion of lead and magnesium that they will have a melting point below 500° C. All lead-magnesium alloys containing up to about 13% magnesium and all such alloys containing between about 28.5 to 47% magnesium 5 have melting points below 500° C. and fall within the broader aspects of our invention. However, it will generally be desirable to use lead-magnesium alloys containing not more than 8.7% of magnesium as these alloys will melt at temperatures not higher than about 400° C. and hence are more convenient to employ. Furthermore, magnesium, up to approximately 5% is 10 very soluble in lead at the molten temperature of 327° C. Therefore, a homogeneous mixture of magnesium in the desired amount of lead-sodium alloy can be obtained by first dissolving the required amount of magnesium in the molten lead before adding to the sodium or before adding the sodium to the molten lead-magnesium alloy. 15 This latter method appears to be the simplest and most practical and is the preferred method of practicing our invention.

In order to more clearly illustrate our invention and the preferred modes of carrying the 20 same into effect, the following examples are given:

*Example 1*

1000 lbs. of molten sodium were gradually 35 added to 8900 lbs. of molten lead at 400° C. A lead-magnesium alloy containing 5% magnesium was melted and 100 lbs. thereof was added to the lead-sodium alloy at 400° C., with stirring. A homogeneous lead-sodium-magnesium 40 alloy containing 10% sodium, 0.05% magnesium and 89.95% lead was obtained.

*Example 2*

45 The same process employed in Example 1 was followed except that only 7000 lbs. of lead were employed and 2000 lbs. of the lead-magnesium alloy was added thereto. The resulting product contained 10% sodium, 89% lead and 1% magnesium.

*Example 3*

1000 lbs. of molten sodium was added to 8985.7 50 lbs. of molten lead at 400° C. The resulting lead-sodium alloy was maintained at 400° C. while 14.3 lbs. of a lead-magnesium alloy containing 35% magnesium was added thereto. The resulting alloy contained 10% sodium, 0.05% magnesium and 89.95% lead.

60

*Example 4*

A mixture of 1000 lbs. of sodium and 8714 lbs. of lead was prepared and maintained at a temperature of 400° C., while to it was added 286 lbs. of a molten lead-magnesium alloy containing 35% of magnesium. The product contained 10% sodium, 1% magnesium and 89% lead.

*Example 5*

5 lbs. of magnesium were dissolved in 8995 lbs. of lead at 327° C. The molten lead-magnesium alloy was then added to 1000 lbs. of molten sodium with stirring. The resulting product contained 10% sodium, 0.05% magnesium and 89.95% lead.

*Example 6*

100 lbs. of magnesium were dissolved in 8900 10 lbs. of lead at 327° C. To this was added 1000 lbs. of molten sodium with stirring and without permitting the temperature to rise above 400° C. The resulting product contained 10% sodium, 15 1% magnesium, and 89% lead.

While we have disclosed the preferred embodiments of our invention, it will be readily apparent to those skilled in the art that many variations and modifications may be made therein without departing from the spirit thereof. Accordingly, the scope of our invention is to be limited solely by the appended claims, construed as broadly as is permissible in view of the prior art.

We claim:

1. The process of preparing an alloy comprising 10% sodium, 89.95% to 89.00% lead and 0.05% to 1.00% magnesium which comprises fusing the magnesium with sufficient molten lead to produce a mixture melting below 500° C. and then fusing the mixture with sufficient sodium and lead to produce the alloy, the magnesium being fused with the lead at temperatures below the melting point of the magnesium and the lead-magnesium mixture being fused with the sodium at temperatures below 500° C. and above the melting point of said mixture.

2. The process of preparing an alloy comprising 10% sodium, 89.95% to 89.00% lead and 0.05% to 1.00% magnesium which comprises 40 fusing the magnesium with at least 90% of the molten lead and then fusing the mixture with sufficient sodium and lead to produce the alloy, the magnesium being fused with the lead at temperatures below the melting point of the magnesium and the lead-magnesium mixture being fused with the sodium at temperatures below 500° C. and above the melting point of said mixture.

3. The process of preparing an alloy comprising 10% sodium, 89.95% to 89.00% lead and 0.05% to 1.00% magnesium which comprises fusing the magnesium with the molten lead and then fusing the mixture with the sodium, the magnesium being fused with the lead at temperatures below the melting point of the magnesium and the lead-magnesium mixture being fused with the sodium at temperatures below 500° C. and above the melting point of said mixture.

4. The method of preparing an alloy comprising 10% sodium, 89.95% to 89.00% lead and 0.05% to 1.00% magnesium which comprises fusing the magnesium with the lead at about 327° C. and then adding the sodium while maintaining the temperature to below about 400° C.

FREDERICK BAXTER DOWNING  
LOUIS SAMUEL BAKE,  
ALFRED E. PARMELEE.